# EUROPEAN PATENT SPECIFICATION

(11) **EP 0 552 554 B1**
(45) Date of publication and mention of the grant of the patent: **05.03.1997**
(21) Application number: 92311497.9
(22) Date of filing: 16.12.1992
(51) Int. Cl.: C10M 105/00, C10M 111/02, C10M 169/04

(54) **Lubricating oil compositions**
Schmierölzusammensetzungen
Compositions d'huile lubrifiante

(30) Priority: 22.01.1992 GB 9201338
(43) Date of publication of application: 28.07.1993
(73) Proprietor: THE BRITISH PETROLEUM COMPANY P.L.C., London EC2M 7BA (GB)
(72) Inventor: Holt, Grenville, London EC2Y 7BU (GB); Murray, Bruce Lawrence John, London EC2Y 7BU (GB)
(74) Representative: Krishnan, Suryanarayana Kalyana

(56) References cited:
- EP-A- 0 259 809
- EP-A- 0 468 109
- DE-A- 1 594 641
- DE-A- 1 913 538
- FR-A- 2 195 674
- GB-A- 1 131 926
- US-A- 3 974 081

## Description

The present invention relates to environmentally friendly lubricating oil compositions for automotive engines. Lubricating oil compositions for use in automotive engines are well known. EP-A-0 259 809 discloses, a lubricating oil composition comprising 97 to 60% by weight of mineral oil and 3 to 40% by weight of polyester, said mineral oil having a dynamic viscosity at 100°C of 2 to 50 centistokes, a pour point ( as determined by JIS K-2269) of -5 to -30°C, a viscosity index (as determined by JIS K-2283) of not less than 80 and % C_{A} of not more than 3. This lubricating oil composition is suitable for lubrication of parts including a wet brake and a wet clutch, such as automatic transmissions and tractors. These compositions usually contain a base fluid which may comprise mineral oils, hydrocarbon oils and/or synthetic fluids and conventional additives such as viscosity index (hereafter "VI") improvers, anti-oxidants, corrosion inhibitors, dispersants, anti-wear additives and sludge control agents. In recent years, automotive engine oil development has seen a steady trend towards lower viscosity multigrades, principally to improve fuel efficiency. The predominant viscosity grade has moved from a typically 20W/50 oil to a 10W/40 or a 5W/40 oil. The manufacturers of automotive engine equipment have also tightened the specifications for such oils in terms of oil consumption, bearing protection and shear stability. This has meant that the engine lubricant has had to become lower in volatility and more shear stable so that these thinner oils stay in the specified grade band longer. As a result, lubricating oils compositions based solely on conventional solvent refined mineral oils are no longer adequate to meet these stringent performance requirements. To meet these performance requirements, a growing demand has arisen for "special" base oils possessing superior qualities of volatility, VI and pour point. These special base oils have a VI above 120 and the requirement is primarily met by the use of paraffinic base oils which include inter alia oils based on hydrocracked wax distillates. It has also been suggested to use blends of such hydrocracked wax distillates with aliphatic esters in order to improve the performance of such base oils. These prior art compositions usually contain 80%w.w or more of a hydrocarbon or mineral oil and upto 20%w/w of an aliphatic carboxylic acid ester in the base fluid. Such compositions, whilst being very efficient and being to some extent biodegradable, still leave room for improvement.

It has now been found that base oil blends can be formulated which not only improve the biodegradability thereof but achieve the same without loss of performance at the same time exhibiting relatively lower emissions, lower fuel consumption and lower oil consumption.

Accordingly, the present invention is an automotive engine lubricating oil composition which has a major proportion of a base fluid which fluid comprises a blend of:
a) isotridecyl dodecanedioate
b) at least one hydrocarbon oil comprising upto 99.5%w/w of aliphatic hydrocarbons and no more than 10%w/w aromatic hydorcarbons such that the total of aliphatics and aromatics is 100% wherein the amount of component (a) in the blend is in the range from 25-55%w/w.

As described above, the base fluid comprises a blend of an ester and a hydrocarbon oil. The ester component (a) is derivable by the reaction of an aliphatic mono-, di-and/or poly-carboxylic acid with, isotridecyl alcohol under esterification conditions.

Specific examples of such esters include the isotridecyl esters of octane-1,8-dioic acid, 2-ethylhexane-1,6-dioic acid and dodecane-1,12-dioic acid.

Similarly, the hydrocarbon oil component (b) in the blend suitably is a hydrocracked wax distillate. More specifically, such hydrocarbon oils can contain upto 99.5%w/w, preferably upto 97%w/w, of aliphatic hydrocarbons and no more than 10%w/w of aromatic hydrocarbons. The expression "aliphatic hydrocarbons" as used herein and throughout the specification is meant to include open chain aliphatic hydrocarbons as well as cycloaliphatic hydrocarbons such as e.g. naphthenic hydrocarbons. The total polycyclic aromatic hydrocarbons in the hydrocarbon oil is suitably less than 10 ppm, preferably less than 5 ppm and more preferably less than 1 ppm. Typically such hydrocarbon oil contains from 92-97% w/w of aliphatics and 3-8% w/w of aromatics.

The hydrocarbon oil component (b) in the blend is suitably prepared by feeding a waxy distillate through a hydrocracker at 70-95% conversion under elevated temperature and hydrogen pressure. In the first stage of this hydrocracker, sulphur and nitrogen compounds are removed and in the second stage the aromatics are hydrogenated to naphthenes; the hydrogenated products including the naphthenes are cleaved and rearranged to produce a controlled range of paraffins and isoparaffins. Fuels and lubricant products are separated by atmospheric distillation from the resultant hydrocracked products and the 5-35% heavy component is the hydrocarbon fraction used as the hydrocarbon oil component (b) in the blend. A product produced by this method is substantially free of any unsaturates. This feedstock can be further refined, if necessary, by conventional techniques such as additional fractionation, extraction or dewaxing to obtain the finished product. The resultant hydrocarbon oil has the following physical characteristics:

Of the aliphatic hydrocarbons in this hydrocarbon oil component (b), about 20% w/w comprises isoparaffins having an average carbon number of about 27.

The relative amounts of the ester component (a) and the hydrocarbon oil component (b) in the base fluid within the specified ranges above will depend upon the nature of the two components and their relative viscosities. For instance, if the hydrocarbon component (b) is within the physical characteristic specification defined above, and the ester component (a) is isotridecyldodecanedioate, the amount of ester (a) in the blend may suitably vary from 30-50% w/w, preferably from 40-50% w/w.

In addition to the above blended base fluid, the lubricating composition of the present invention comprises minor proportions of conventional additives which include inter alia the following: one or more sludge dispersants, one or more VI improvers, one or more anti-wear additives, and one or more anti-oxidants. Typically, the additive package used is known to comprise components which meet the stringent requirements of an API Performance Classification "SG". These requirements include successful testing in the following categories: rust test, dispersancy test, piston varnish test, low temperature sludge test and wear test. Such additives are commercially available as an additives package sold e.g. as an "SG Additive Package" under the names GBX 2900 and GBX 2905 (both ex Adibis Ltd, UK). Such an additive package suitably forms from 10-20% w/w, preferably from 11-16% w/w of the formulated lubricating composition. Examples of compounds that may be present in such a package include anti-rust agents such as the overbased calcium or magnesium sulphonates or phenates; anti-wear agents such as the zinc dithiophosphates, preferably the zinc dialkyl dithiophosphates containing 5-15% w/w phosphorus (normally prepared using a mixture of secondary alcohols and representing 0.05% -0.5% w/w of phosphorus, typically 0.1-0.14% phosphorus in the finished oil); ashless dispersancy agents such as derivatives of long chain hydrocarbon substituted succinimides, especially the polyisobutenyl succinimides; and sludge dispersants which are oil soluble salts such as amides, imides, oxazolines and esters of mono- or di-carboxylic acids or anhydrides.

The anti-oxidants typically contain phenolic compounds and a typical antioxidant is commercially available as ADX 545A (ex Adibis Ltd). The anti-oxidants are suitably present in an amount from 0.01-5% w/w, preferably from 0.1-2.0% w/w of the formulated lubricating composition.

The lubricating compositions also contain one or more VI improvers. Examples of such VI improvers include polymethacrylate type dispersants commercially sold as Plexol 1420 VX (Regd Trade Mark, ex Rohm GmbH) and hydrotreated polyisoprenes commercially sold as Shellvis 200 (Regd Trade Mark, ex Shell UK Ltd). In the case of the latter, it may used as a solution in the hydrocarbon oil component (b) above. The VI improvers are suitably present in an amount from 2 to 5% w/w of the formulated lubricating composition. Thus a typical formulated lubricating composition (A) can be represented by the following components in w/w %:

| | |
|---|---|
| SG Additives Package (GBX 2905, ex Adibis Ltd) | - 15.4 |
| ADX 545A (anti-oxidant, ex Adibis Ltd) | - 1.0 |
| Plexol* 1420 (VI improver, ex Rohm GmbH) | - 3.1 |
| Shellvis* 200 (VI improver, 10% soln, ex Shell UK Ltd) | - 6.0 |
| Isotridecyldodecanedioate | - 22.59 and |
| Hydrocarbon oil** | - 52.71 |

| | |
|---|---|
| * Registered Trade Mark | |
| ** The hydrocarbon oil is a hydrotreated wax distillate containing 92.3% w/w aliphatics and 7.7% w/w aromatics which is substantially free of any unsaturates and had a polycyclic aromatic content of about 0.1 ppm. An oil of this type is described above. | |

Variations of the formulated lubricating composition (A) shown above can also be formulated in which the relative amounts of ester and hydrocarbon oil are (B) 32.28% and 49.32% respectively or (C) 39.5% each.

It was found that the performance of the lubricating compositions formulated in this manner upon engine testing showed relatively lower emissions, lower fuel consumption, lower oil consumption and low nitrogen oxides emission. In addition, the formulated lubricating compositions according to the present invention were at least 80% biodegradable as measured by the CEC standard test procedure. The present invention is further illustrated with reference to the following Examples:

### Examples - General

A base fluid was prepared using isotridecyldodecanedioate, and a hydrocracked wax distillate having the following physical characteristics:

| Property | Typical Specification | Test Method |
|---|---|---|
| Colour | 1.5 max | ASTM D 1500 |
| Density | 0.83 | ASTM D 1298 |
| KV 40/cSt | 17.28 | ASTM d 445 |
| KV 100/cSt | 3.99 | ASTM d 445 |
| VI | 128 | ASTM D 2270 |
| PMC/°C | 220 | ASTM D 93 |
| Pour Point | -27 | ASTM D 97 |
| Demulse/mins | <5 | NFT* 60-125 |
| Noack volatility/% | 15.8 | DIN 51581 |
| Sulphur/% | 0.08 | XRF NFM 07053 |
| CA/% | 2 | Brandes Method |

| | | |
|---|---|---|
| *Correlates with ASTM D 1401 | | |

This hydrocarbon oil was used to prepare formulated lubricating oil compositions according to the formulation in (A) in the following Examples 1-3.

### Example 1

| | |
|---|---|
| SG Additive Package (GBX 2905, ex Adibis Ltd) | - 15.4% w/w |
| ADX 545A (Anti-oxidant, ex Adibis Ltd) | - 1.0% w/w |
| Plexol* 1420 (VI improver, ex Rohm GmbH) | - 3.1% w/w |
| Shellvis* 200 (VI improver, 10% solution, ex Shell UK Ltd) | - 6.0% w/w |
| Isotridecyl dodecanedioate | - 22.59% w/w |
| Hydrocarbon oil (as above) | - 52.71% w/w |

| | |
|---|---|
| *Registered Trade Mark | |

The formulation was prepared using standard lubricant blending techniques described e.g. in "Lubricants and Related Products" by D Klamann, published by Verlag Chemie, 1984.

The formulated composition had the following characteristics:

| Property | Limits | Methods |
|---|---|---|
| Viscosity @ 100°C | 13.6-14.5 cSt | ASTM D 445 |
| Viscosity @ 40°C | 75.0-83.0 cSt | ASTM D 445 |
| Viscosity @ -25°C | <3500 cP | ASTM D 2602 |
| Noack volatility | 8.5-11.0% | DIN 51581 |
| Biodegradability | >80% | CEC-L-33-T-82 |
| Calcium | 0.300-0.332 | ICP |
| Phosphorus | 0.102-0.114 | ICP |
| Zinc | 0.105-0.135 | ICP |

### Example 2

| | |
|---|---|
| SH Additive Package (eg OS 99099, ex Lubrizol Ltd) | - 15% w/w |
| Viscoplex* 2540 (VI Improver, ex Rohm GmbH) | - 3.0% w/w |
| Shellvis* 201 (VI Improver, ex Shell UK Ltd) | - 3.8% w/w |
| Isotridecyl dodecanedioate | - 38.1% w/w |
| Hydrocarbon oil (as above) | - 40.1% w/w |

| | |
|---|---|
| *Registered Trade Mark | |

The formulated composition had the following characteristics:

| Property | Limits | Method |
|---|---|---|
| Viscosity @ 100°C | 14.0 cSt | ASTM D445 |
| Viscosity @ -25°C | 3200 cP | ASTM D2602 |
| Noack volatility | 10.7% | DIN 51581 |
| Biodegradability | 87% | CEC-L-33-T-82 |
| Calcium content | 0.283 | ICP |
| Phosphorus content | 0.119 | ICP |
| Zinc content | 0.128 | ICP |

### Example 3

| | |
|---|---|
| SG Additive Package (eg GBX2905, ex Adibis Ltd) | - 16.4% w/w |
| Plexol* 1420 (VI Improver, ex Rohm GmbH) | - 3.1% w/w |
| GBX 2715 (VI Improver, ex Adibis Ltd) | - 5.0% w/w |
| Isotridecyl dodecanedioate | - 40.0% w/w |
| Hydrocarbon oil (as above) | - 35.5% w/w |

| | |
|---|---|
| *Registered Trade Mark | |

The formulated composition had the following properties:

| Property | Limits | Method |
|---|---|---|
| Viscosity @ 100°C | 14.5 cSt | ASTM D445 |
| Viscosity @ -25°C | 3300 cP | ASTM D2602 |
| Noack volatility | 10.4% | DIM 51581 |
| Biodegradability | 86% | CEC-L-33-T-82 |
| Calcium content | 0.310% | ICP |
| Phosphorus content | 0.108% | ICP |
| Zinc content | 0.125% | ICP |

Upon standard engine testing each of the formulations described in Examples 1-3 above using the API-GS method, the following properties were observed:

| Property | Performance |
|---|---|
| Volatility | Good |
| Low Temperature | Good |
| Oxidation Stability | |
| Industrial | Very Good |
| Automotive | |
| 10W/40 | Very Good |
| 5W/40,50 | Good |
| Detergency | |
| 10W/40 (a) | Very Good |
| 10W/40 (b) | Very Good |
| Dispersancy | |
| 10W/40 | Very Good |
| 5W/40,50 | Very Good |
| Seal Compatibility | |
| 10W/40 (a) | Good |
| 10W/40 (b) | Good |
| Wear/Friction | |
| 10W/40 (a) | Very Good |
| 10W/40 (b) | Very Good |
| 5W/40,50 | Very Good |
| Additive Solubility | Good |

The biodegradability of the formulated lubricating composition according to the present invention was tested and compared with commercially available products using the test method shown in the table above. The results are tabulated below:

| | |
|---|---|
| Present Invention | 91% |
| Mobil 1 | 45% |
| Castrol GTX | 63% |
| Shell Gemini | 66% |
| Castrol Syntron | 41% |

From the above it is clear that the formulated compositions according to the present invention containing the blended base fluid according to the present invention show superior properties to those of prior art, especially in respect of their biodegradability.

## Claims

1. An automotive engine lubricating oil composition which has a major proportion of a base fluid which fluid comprises a blend of:
a) isotridecyl dodecanedioate, and
b) at least one hydrocarbon oil comprising up to 99.5%w/w of aliphatic hydrocarbons and no more than 10%w/w of aromatic hydrocarbons such that the total of aliphatics and aromatics is 100%, wherein the amount of component (a) in the blend is in the range from 25-55%w/w.

2. A lubricating oil composition according to claim 1 wherein the hydrocarbon oil component (b) is a hydrocracked wax distillate.

3. A lubricating oil composition according to claim 1 or claim 2 wherein the hydrocarbon oil component (b) contains less than 10ppm of polycyclic aromatic hydrocarbons, from 92-97%w/w of aliphatic hydrocarbons and 3-8%w/w of aromatic hydrocarbons.

4. A lubricating oil composition according to any one of the preceding claims wherein the aliphatic hydrocarbons in the hydrocarbon oil component (b) comprise about 20%w/w of isoparaffins having an average carbon number of about 27.

5. A lubricating oil composition according to any one of the preceding claims wherein the isotridecyl dodecanedioate is present in the blend in the range from 30-50%w/w.

6. A lubricating oil composition according to any one of the preceding claims wherein said composition comprises, in addition, minor proportions of one or more additives selected from: sludge dispersants, ashless dispersancy agents, VI improvers, anti-wear additives, anti-rust agents and anti-oxidants.

7. A lubricating oil composition according to claim 6 wherein the anti-rust agent is an overbased calcium or magnesium sulphonate or phenate; the anti-wear agent is a zinc dithiophosphate; the ashless dispersancy agent is a long chain hydrocarbon substituted succinimide; the sludge dispersant is an oil soluble salt such as amides, imides, oxazolines and esters of mono- or di-carboxylic acids or anhydrides; the anti-oxidant is a phenolic compound; and the VI improver comprises a polymethacrylate dispersant or a hydrotreated polyisoprene.

8. A lubricating oil composition according to any one of the preceding claims wherein said composition is at least 80% biodegradable as measured by the CEC-L-33-T-82 standard test procedure.

## Patentansprüche

1. Schmierölzusammensetzung für Kraftfahrzeugmotoren, die als Hauptanteil eine Grundflüssigkeit aufweist, wobei die Flüssigkeit ein Gemisch umfaßt von:
a) Dodecandisäurediisotridecylester und
b) mindestens einem Kohlenwasserstofföl, umfassend bis zu 99,5% Gewicht/Gewicht aliphatische Kohlenwasserstoffe und nicht mehr als 10% Gewicht/Gewicht aromatische Kohlenwasserstoffe, so daß aliphatische und aromatische Stoffe insgesamt 100% sind, wobei die Menge an Komponente (a) in dem Gemisch im Bereich 25-55% Gewicht/Gewicht liegt.

2. Schmierölzusammensetzung nach Anspruch 1, wobei die Kohlenwasserstoffölkomponente (b) ein hydrogecracktes Wachsdestillat ist.

3. Schmierölzusammensetzung nach Anspruch 1 oder Anspruch 2, wobei die Kohlenwasserstoffölkomponente (b) weniger als 10 ppm polycyclische aromatische Kohlenwasserstoffe, 92-97% Gewicht/Gewicht aliphatische Kohlenwasserstoffe und 3-8% Gewicht/Gewicht aromatische Kohlenwasserstoffe enthält.

4. Schmierölzusammensetzung nach einem der vorangehenden Ansprüche, wobei die aliphatischen Kohlenwasserstoffe in der Kohlenwasserstoffölkomponente (b) etwa 20% Gewicht/Gewicht Isoparaffine mit einer mittleren Kohlenstoffatomzahl von etwa 27 umfassen.

5. Schmierölzusammensetzung nach einem der vorangehenden Ansprüche, wobei der Dodecandisäurediisotridecylester in dem Gemisch im Bereich 30-50% Gewicht/Gewicht vorliegt.

6. Schmierölzusammensetzung nach einem der vorangehenden Ansprüche, wobei die Zusammensetzung zusätzlich geringe Anteile eines oder mehrerer Additive umfaßt, ausgewählt aus: Schlammdispersants, aschefreien Dispergiermitteln, VI-Verbesserern, Antiverschleißadditiven, Antirostadditiven und Antioxidantien.

7. Schmierölzusammensetzung nach Anspruch 6, wobei das Antirostmittel ein überbasisches Calcium- oder Magnesiumsulfonat oder -phenolat ist; das Antiverschleißmittel ein Zinkdithiophosphat ist; das aschefreie Dispergiermittel ein langkettiges Kohlenwasserstoff-substituiertes Succinimid ist; der Schlammdispersant ein öllösliches Salz, wie Amide, Imide, Oxazoline und Ester von Mono- oder Dicarbonsäuren oder -anhydriden ist; das Antioxidans eine Phenolverbindung ist und der VI-Verbesserer einen Polymethacrylat-Dispersant oder ein hydrobehandeltes Polyisopren umfaßt.

8. Schmierölzusammensetzung nach einem der vorangehenden Ansprüche, wobei die Zusammensetzung mindestens 80% bioabbaubar ist, gemessen durch den CEC-L-33-T-82-Standardtestvorgang.

## Revendications

1. Composition d'huile lubrifiante pour moteur d'automobile qui possède une proportion principale d'un fluide de base, lequel fluide comprend un mélange:
a) de dodécanedioate d'isotridécyle et
b) d'au moins une huile hydrocarbonée comprenant jusqu'à 99,5% p/p d'hydrocarbures aliphatiques et pas plus de 10% p/p d'hydrocarbures aromatiques de sorte que le total des substances aliphatiques et aromatiques fasse 100% dans laquelle la quantité de composant (a) dans le mélange est comprise entre 25 et 55% p/p.

2. Composition d'huile lubrifiante selon la revendication 1, dans laquelle le composant (b) d'huile hydrocarbonée est un distillat de cire hydrocraquée.

3. Composition d'huile lubrifiante selon la revendication 1 ou la revendication 2 dans laquelle le composant (b) d'huile hydrocarbonée contient moins de 10 ppm d'hydrocarbures aromatiques polycycliques, de 92 à 97% p/p d'hydrocarbures aliphatiques et 3 à 8% p/p d'hydrocarbures aromatiques.

4. Composition d'huile lubrifiante selon l'une des revendications précédentes, dans laquelle les hydrocarbures aliphatiques dans le composant (b) d'huile hydrocarbonée comprennent environ 20% p/p d'isoparaffines ayant un nombre d'atomes de carbone moyen d'environ 27.

5. Composition d'huile lubrifiante selon l'une des revendications précédentes, dans laquelle le dodécanedioate d'isotridécyle est présent dans le mélange en quantité comprise entre 30 et 50% p/p.

6. Composition d'huile lubrifiante selon l'une des revendications précédentes dans laquelle ladite composition comprend, de plus, des proportions mineures d'un ou plusieurs additifs choisis parmi: les dispersants de boue, les agents de dispersion sans cendre, les agents d'amélioration de la viscosité, les additifs anti-usure, les agents antirouille et les anti-oxydants.

7. Composition d'huile lubrifiante selon la revendication 6, dans laquelle l'agent antirouille est le sulfonate ou le phénate de calcium ou de magnésium; l'agent anti-usure est un dithiophosphate de zinc, l'agent de dispersion sans cendre est un succinimide substitué par une longue chaîne hydrocarbonée; le dispersant de boue est un sel liposoluble tel que les amides, les imides, les oxazolines et les esters des acides ou anhydrides mono- ou di-carboxyliques; l'antioxydant est un composé phénolique; et l'agent d'amélioration de VI comprend un dispersant à base de polyméthacrylate ou un polyisoprène hydrotraité.

8. Composition d'huile lubrifiante selon l'une des revendications précédentes dans laquelle ladite composition est biodégradable au moins à 80% tel que mesuré par le procédé d'essai normalisé CEC-L-33-T-82.
